

Jan. 27, 1942.

W. HESTERMANN

2,270,845

PROTECTIVE LINING FOR METAL CONTAINERS

Filed June 27, 1939

*Fig. 1.*



*Fig. 2.*



INVENTOR.

WALTER HESTERMANN.

BY

Benj. T. Pauber ATTORNEY.

## UNITED STATES PATENT OFFICE

2,270,845

## PROTECTIVE LINING FOR METAL CONTAINERS

Walter Hestermann, Jersey City, N. J., assignor  
to White Metal Manufacturing Company,  
Hoboken, N. J., a corporation of New Jersey

Application June 27, 1939, Serial No. 281,343

4 Claims. (Cl. 221—60)

My invention relates to a protective coating for rendering the inner surface of metal containers, particularly collapsible tubes, more resistant to corrosion or attack by the substances contained within the container.

Collapsible tubes are generally formed of tin, lead or aluminum, or of suitable alloys of these metals, or of composite metals, such as lead coated with tin. The tubes are usually manufactured by extrusion from blanks of the metal. The walls of the tubes must, of necessity, be thin and flexible.

Tubes of the above type are used as containers for materials of a wide variety of chemical compositions. Some of the substances may be alkaline in reaction, particularly under certain conditions, while others may be acid, and others contain various salts, solvents or diluents. Consequently these materials may react deleteriously with the inner surface of the tube, occasionally eating through the relatively thin walls thereof in one or more spots or areas and forming compounds therewith which either discolor the contents of the tube, or which may even be toxic, or semi-toxic, when absorbed by the tube contents.

Owing to the wide variation in the characteristics of the materials that may fill the tubes, and to the fact that the tubes may be stored under a wide variety of conditions, it is very difficult to protect the inner surfaces of the tubes by a protective lining. Such a lining or coating in order to be effective, must not only be flexible, but must adhere well to the surfaces of the tubes, be free from cracks or defects and must resist attack or dissolution by any of the various materials filling the tubes under the wide variety of conditions in which the tubes may be stored. For example, certain materials may be relatively inactive towards the coating at ordinary temperatures and when air is excluded, but may be more reactive if air is present, or if the temperature is high, or if suitable conditions of temperature or of humidity are present. For example, a filling material that might not attack the lining within the ordinary period of storage and use in a cold or temperature climate, might be much more reactive in the tropics; or, if a small amount of air were enclosed during filling, this might cause an attack on the lining and of the tube itself during storage, transportation and sale in a hot or tropical country. The resultant loss due to the failure of even a very small percentage, or fraction of a per cent, is of course a serious matter because not only is the tube itself

lost but its contents besides, creating considerable expense and, possibly, loss of sales.

My present invention provides a tube lining or coating of greatly increased resistance to the contents of tubes as, for example, shaving cream or shaving soap, and which resists attack by corrosive materials or fillings for an extended period of time, and thereby effectively protects the walls of the tube from corrosion even under adverse circumstances.

In my present invention I coat the inner surface of the tube with a solution of alkyl cellulose as, for example, ethyl cellulose made by the reaction of alkali cellulose and ethyl chloride together with a suitable plasticizer and solvent. As an example of a coating formed in accordance with my invention, I dissolve ethyl cellulose in a suitable solvent. Solvents for ethyl cellulose are certain alcohols, alcoholic ethers, aromatic hydrocarbons, petroleum hydrocarbon, or mixtures of them. For example, a suitable mixture is one containing the following:

|                             | Parts |
|-----------------------------|-------|
| Toluene                     | 4     |
| Ethanol                     | 1     |
| Xylo (or petroleum spirits) | 4     |
| Butyl alcohol               | 1     |

The ethyl cellulose is dissolved in the above solvent mixture in quantities to produce a finished product having approximately 7 to 7½% solids.

In order to obtain an increased adhesion and flexibility, a small amount of a plastic material is added. Bakelite or other natural, or artificial resins or gums may be employed as plasticizers. However, I prefer to use an ester of a polyhydric alcohol and a dibasic acid. Glycol sebacate is a very desirable ester for this purpose. However, esters of succinic, glutaric, adipic acid, etc., and other dibasic acids may be employed. Glycol sebacate has sticky, non-drying characteristics which are retained in the resulting lacquer to a sufficient extent to ensure good adhesion to the wall of the tube and with continued flexibility of the coating so that it will bend with the wall of the tube without cracking or breaking. An amount of glycol sebacate (known in the trade as "Faraplex") equal to 2% to 3% by weight of the ethyl cellulose is sufficient for this purpose.

To form the coating, the tube is sprayed or covered with a thin film of the solution of ethyl or alkyl cellulose and then permitted to dry.

An example of such a tube is shown in the accompanying drawing, in which—

Fig. 1 is a vertical section of a tube, and

Fig. 2 is a cross section on a larger scale on the line 2--2 of Fig. 1.

In these figures, the wall of the tube is represented as 1 and the coating 2. A thin film of the above coating when dry, protects the inner surface of the tube from corrosion by acids or alkalies, or acid reacting materials, and from deleterious contact with various salts and solvents that may be present in the contents of the container. The coating greatly increases the life of tubes, and particularly of tubes made of lead, lead alloy, 10 tin, and lead coated with tin. In the case of tin coated lead tubes, the tin is not always distributed uniformly over the lead surface, and occasionally the lead is exposed at isolated points 15 or in streaks or areas. Occasionally also, the tin surface layer is relatively thin and does not afford a long lived protection against exposure of the lead. The lead must, however, be kept from contact with the contents of the tube.

A coating formed of an alkyl cellulose, such as ethyl cellulose, protects the surface of the tube for a much longer period of time than other coatings or lacquers. A 10% soap solution in contact with air is highly destructive to such a lacquer as alkali-resistant pyroxylin. A tube 25 coated with pyroxylin and inverted and filled to within a short distance of its top edge with a 10% soap solution began to fail after 72 hours, and failed completely within 120 hours. This is, of course, equivalent to a matter of months for a soap paste not exposed to air. However, 30 a tube coated with the coating of the present invention and of equal thickness, did not begin

to fail until it had been exposed under the same conditions as the 10% soap solution, for a period of 150 to 200 hours. The thickness of the coating was about .001 of an inch in each case.

It will be apparent, of course, that ethyl cellulose is given merely by way of example because it is the most convenient, and that other alkyl cellulose may be employed as, for example, butyl, propyl, etc., cellulose when they are available.

Through the above invention, therefore, I have provided a lining or coating for metal containers, such as collapsible tubes, which is very resistant to attack by the contents of the tubes, and which effectively protects the walls of the tubes against corrosion.

What I claim is:

1. A collapsible tube having a flexible adherent inner coating comprising an alkyl cellulose containing not over about 3% of its weight of glycol sebacate.

2. A collapsible tube having a flexible adherent inner coating comprising an ethyl cellulose containing not over about 3% of its weight of glycol sebacate.

3. A collapsible tube having a flexible adherent inner coating comprising an alkyl cellulose containing not over about 3% of its weight of an ester of sebacic acid and a polyhydric alcohol.

4. A collapsible tube having a flexible adherent inner coating comprising an ethyl cellulose containing not over about 3% of its weight of an ester of sebacic acid and a polyhydric alcohol.

WALTER HESTERMANN.